

1,624,071

April 12, 1927.

H. K. RICHARDSON

METHOD OF AFFIXING COATINGS ON INCANDESCENT LAMP FILAMENTS.

Filed July 28, 1921

FIG. 1.



FIG. 3.



FIG. 2.

INVENTOR  
HENRY K. RICHARDSON

BY  
*J. T. Lebort*  
ATTORNEY

## UNITED STATES PATENT OFFICE.

HENRY KNEELAND RICHARDSON, OF EAST ORANGE, NEW JERSEY, ASSIGNOR TO  
WESTINGHOUSE LAMP COMPANY, A CORPORATION OF PENNSYLVANIA.

## METHOD OF AFFIXING COATINGS ON INCANDESCENT-LAMP FILAMENTS.

Application filed July 28, 1921. Serial No. 488,133.

This invention relates to processes of combining rare earths, alkaline earths or oxides with metals and, more particularly, it relates to the application of such earths 5 to incandescent lamp filaments.

An object of the invention is the provision of a novel method for firmly affixing a coating of a rare earth or an alkaline earth to electrical conductors, such as lamp 10 filaments, electrodes, etc.

Another object of the invention is to so affix a coating of an earth to a lamp filament that it may not readily be removed.

Other objects of the invention will be 15 apparent from a reading of the following description.

Heretofore, in the incandescent lighting art, it has been found advantageous to combine rare and alkaline earths with certain 20 glowers, such as lamp filaments, to increase their efficiency and to obtain certain lighting effects. In combining the earths with the filaments, certain difficulties have developed and especially where such earths 25 have been applied as coatings, as, under operation, they have cracked and broken off. The present invention has to do with a new method for firmly affixing earths, as coatings, to lamp filaments.

30 In the accompanying drawings, illustrating an apparatus for carrying out my invention;

Fig. 1 is a diagrammatic illustration of an apparatus for practicing the method;

35 Fig. 2 is a diagrammatic illustration of a modified form of apparatus; and

Fig. 3 is a side elevation of a lamp employed in the apparatus for coating filaments which are later to be sealed in other 40 lamps.

In the drawings, and particularly in Fig. 1, is shown an incandescent lamp 1 comprising an evacuated envelope 2 having a filament 3 mounted therein. The degree of 45 vacuum in the envelope ranges from 1 to 100 microns to efficiently practice the invention. Although coatings may be affixed when the vacuum varies above or below the range indicated, the results obtained under such conditions are imperfect. A small amount of 50 a selected earth 4 is introduced into the envelope 2 before the filament 3 is sealed

therein. The earth is employed in its powdered form and it is found that, as the fineness thereof increases, the coating is 55 more readily and uniformly affixed. The earth may be an oxide of any one of the following metals: Calcium, cerium, barium, thorium, strontium, or yttrium; or a mixture of two or more of the earths mentioned.

Any suitable apparatus may be employed for impressing a high potential between the filament 3 and an exterior electrode 5 of substantial area, such as a sheet of tin foil, 65 and co-operatively positioned with respect to the earth. The apparatus illustrated has proved satisfactory in practicing my invention and may consist of a direct-current generator 6 connected, through a reversing switch 7, to the primary winding of an induction coil 8 which is provided with an interrupter 9. Electrical conductors 10 and 11, respectively, lead to the filament 3 and the tin-foil electrode 5. In the operation of this apparatus, the high potential derived 70 from the generator and the induction coil is impressed across the electrodes. The voltage impressed upon the electrodes 3 and 5 may be varied within wide limits, satisfactory results having been obtained using from 12,000 to 40,000 volts. In using a direct-current generator as the source of energy, very satisfactory results are obtained by making the tin foil the more positive electrode.

85 It will be understood, that in using an induction coil to generate high potential, an interrupted direct current is delivered to the primary winding and alternating potential 90 is developed in the secondary winding thereof, however the potential developed, although alternating, is biased to some degree, because the induced potential is greater upon breaking the primary circuit than upon making the primary circuit. By specifying that the tin foil is made the more positive electrode, it is intended, as will be obvious, that the electrode 5 is positive 95 upon the breaking of the primary circuit.

100 In the early stage of impressing the high potential, it is noted that, by reversing the direction of the current several times, the coating begins to appear on the filament in

a much shorter time. I have found that the filament may also become coated when alternating current is employed in the primary winding.

5 My experiments have shown that, by impressing high potential across the electrodes, the filament becomes coated with the earth or oxide used. The action between the filament and the earth, in producing the desired result, cannot be completely accounted for in the present knowledge of the art. It is well known that a charged body attracts uncharged particles, and charged bodies attract each other when their charges are 10 unlike in sign, but repel each other when their charges are alike. The operation, according to my invention, may therefore be explained because the particles of earth or oxide are either not charged or charged 15 to a potential different in sign from that of the filament 3 desired to be coated. That is, there is a potential difference between filament 3 and the electrode 5, even though the applied current is alternating. I have 20 demonstrated, after study and experiment, by thorough tests under operating conditions, that filaments coated as stated embody qualities which make them desirable, although it is not definitely known why the 25 oxide sticks so firmly after being attracted to the filament.

The ease with which the earth is deposited may be increased by heating the filament as, for instance, by connecting the filament in 30 series with a battery 12 which may be thrown into or out of the circuit by operating a switch 13.

In Fig. 2 is illustrated a modified form of a lamp employed in successively performing 35 additional experiments. This lamp is provided with a grid 14 instead of a filament and has an electrode 15 sealed in the envelope to take the place of the tin-foil electrode.

In some instances, it is desirable to have 40 the coated filaments mounted in envelopes which do not carry the earth. To that end an open envelope 16 (Fig. 3) is connected in the electrical system illustrated in Fig. 1. The earth to be affixed is placed in the bottom 45 thereof and the filament is held within the envelope by a stem 17 which is carried in a rubber stopper 18. The rubber stopper fills the opening and permits the envelope to be exhausted through the tube 19 in the usual manner, and the high potential is impressed as described above.

The method of affixing a coating to a metal or base has been described in connection with the coating of a filament but it 50 is to be understood that it may be employed in applying earth to electrodes used in various electrical devices.

What is claimed is:

1. The method of affixing a coating of a 55 metallic oxide to an electrode comprising

connecting the electrode, in a rarified atmosphere in the presence of the metallic oxide in powdered form, with an other electrode in an electric circuit, and impressing a high potential between said electrodes to cause a 70 bodily transfer of the powdered particles to the electrode without dissociation thereof.

2. The method of affixing a refractory metallic compound onto a filamentary material in a firmly adherent manner which 75 consists in disposing the filamentary material adjacent said compound in a vacuum and creating an electrical difference of potential of large magnitude between said filamentary material and said compound to 80 effect a bodily transfer of the compound to the filamentary material without dissociation thereof.

3. The method of coating a filament with a firmly adherent deposit of an earth comprising mounting the filament in an envelope having a rarified atmosphere and containing said earth and an electrode which cooperates with said earth and impressing a high potential 85 between the electrode and the filament 90 to cause a bodily transfer of the earth to the filament without dissociation thereof.

4. The method of coating a filament with an earth comprising mounting the filament in an evacuated envelope containing said 95 earth in powdered form, said envelope being provided with an electrode cooperating with said earth, connecting said filament in an electrical circuit, impressing a high potential between said filament and the 100 electrode and subsequently reversing the direction of the applied potential.

5. The method of affixing an earth to a filament comprising mounting the filament in an evacuated envelope having an electrode 105 associated therewith, introducing such earth therein in powdered form, impressing a high potential between said filament and the electrode to cause a bodily transfer of the powdered earth to the filament and heating said 110 filament by independent means.

6. The method of manufacturing oxide-coated filamentary material comprising placing some alkaline earth in powdered form in a vessel adapted to be evacuated, providing an external electrode for said vessel below the alkaline earth, inserting filamentary material into said vessel above the alkaline earth, evacuating said vessel and impressing a high potential between the electrode and 115 the filamentary material.

7. The method of manufacturing oxide-coated filamentary material comprising placing some powdered oxide in a vessel adapted to be evacuated, providing an external electrode for said vessel below the oxide, inserting filamentary material into said vessel about the oxide, evacuating said vessel and impressing a high potential between the 125 electrode and the filamentary material, while 130

maintaining said material in a heated condition, from an independent source of electricity.

8. An electric device comprising an evacuated vessel provided with some earth in powdered form, a filament sealed therein, an electrode cooperating with said earth and means for impressing a high potential be-

tween said electrode and the filament to cause some of said earth to be attracted to 10 the filament and firmly adhere thereto.

In testimony whereof, I have hereunto subscribed my name this 27th day of July, 1921.

HENRY KNEELAND RICHARDSON.